

# United States Patent Office

2,876,096

Patented Mar. 3, 1959

1

2,876,096

## NON-MAGNETIC AUSTENITIC STEEL

Peter Payson, Pittsburgh, Pa., assignor to Crucible Steel Company of America, Pittsburgh, Pa., a corporation of New Jersey

No Drawing. Application December 27, 1957  
Serial No. 705,489

2 Claims. (Cl. 75—126)

This invention pertains to a substantially nickel-free, non-age hardenable and non-magnetic, austenitic steel, which remains non-magnetic on cold working.

It is the object of this invention to provide a substantially non-magnetic, austenitic alloy steel practically free from nickel. Aside from the Hadfield manganese steel, which has limits of usefulness because of fabrication difficulties, all steels now available which are relatively non-magnetic, that is, those which have permeability values under about 1.2 contain appreciable amounts of nickel. Characteristic of these are the austenitic stainless steels, for examples, types 302 (approximately 18% chromium and 8% nickel) and 310 (approximately 25% chromium and 20% nickel). Another important non-magnetic material for electrical equipment contains about .35% carbon, 13% manganese, 8.0% nickel, balance iron.

The low carbon, 16% manganese, 16% chromium, .15% nitrogen steel which is now becoming available as a replacement for type 302 is non-magnetic as annealed, but it becomes appreciably magnetic after it is subjected to some cold working.

The recently developed demand for a non-magnetic, low cost steel for certain types of naval vessels, together with the present limit on availability of nickel for such materials, make it highly desirable to provide a relatively low alloy steel which has the desired non-magnetic property and which is not dependent on nickel for this characteristic. I have invented a steel which meets these requirements, the "broad" and "preferred" ranges of analysis of which are as follows:

| Analysis, Wt. Percent                           | Broad                                               | Preferred                                           |
|-------------------------------------------------|-----------------------------------------------------|-----------------------------------------------------|
| Carbon.....                                     | .30/.45.....                                        | .35/.45.....                                        |
| Manganese.....                                  | 11.0/15.0.....                                      | 12.0/14.0.....                                      |
| Silicon.....                                    | .10 to 1.0.....                                     | .20/.50.....                                        |
| Nickel.....                                     | up to 1.0.....                                      | .50/1.00.....                                       |
| Chromium.....                                   | 11.0/15.0.....                                      | 12.0/13.0.....                                      |
| Nitrogen.....                                   | .15/.60.....                                        | .15/.25.....                                        |
| Other elements including Mo, W, V, Cu, Al, etc. | up to 1.0 total with none exceeding about 0.2%..... | up to 1.0 total with none exceeding about 0.2%..... |
| Balance, Iron.                                  |                                                     |                                                     |

For a ferrous material to be non-magnetic it is necessary that its structure be substantially austenitic at ambient temperatures. To retain the austenitic structure at low temperatures, it is necessary that the steel have

2

in its composition substantial quantities of those elements which are effective in suppressing its Ms temperature or austenite-to-martensite transformation temperature. These are notably carbon, manganese, chromium and nickel as has been established in the publication "Martensite Reactions in Alloy Steels" by P. Payson and C. H. Savage, Trans. A. S. M., vol. 33, 1944, p. 261. Nitrogen is also known to have an appreciable stabilizing effect on austenite in steel.

Since manganese is highly effective in suppressing the martensite reaction, and since it is one of the least expensive steel alloying elements, I depend primarily on this element in the production of my non-magnetic steel. Furthermore, the presence of high manganese in the steel permits relatively large amounts of nitrogen to be dissolved therein which is desirable to attain the objective of a relatively low cost non-magnetic material. I set a minimum of about 11% manganese for the steel of this invention so that I may use relatively low carbon therein. If lower amounts of manganese are used, it is necessary also to employ relatively high carbon in order to stabilize the austenite, and it is further desirable to keep the carbon as low as possible to assure that the weldability of the steel will be at a maximum.

Since most of the manganese in steel is lost in the remelting of scrap, it is preferable not to depend entirely on manganese and carbon to provide stability of the austenite, and up to this time nickel has been depended upon to supplement the manganese in stabilizing the austenite. But I have established that chromium in amounts of about 11 to 15% serves admirably for this purpose. Ordinarily chromium is thought of as a ferrite forming element, which indeed it is when the carbon and nitrogen contents of the steel are low. But when both carbon and nitrogen in the steel are above about a total of 0.30%, a sizeable quantity of chromium, that is, well over 15%, is needed to establish free ferrite in the steel. Another advantage in the use of chromium rather than nickel for stabilizing the austenite in the non-magnetic steel is that chromium like manganese increases the solubility of nitrogen in the steel. The low limit of chromium in the stable non-magnetic steel depends on the amounts of carbon and nitrogen present, in addition to manganese, as will be shown below.

It is well known that semi-stable austenite can be made to transform to a magnetic phase by subjecting it to plastic deformation at room temperature. The relative magnetic susceptibility of the steel after cold working is, therefore, a measure of the stability of the austenite, the lower the susceptibility with more and more cold working, the greater the stability of the steel.

The data in Table I below show the effects of composition on the magnetic susceptibility after cold working of the C—Mn—Cr—N steel containing varying amounts of carbon and nitrogen in addition to chromium:

TABLE I  
Effect of composition and percent cold work on magnetic susceptibility of steels

[All steels were first annealed by an air cool from 1950° F. and were then cold reduced as indicated.]

| Bar       | C   | Mn   | Si   | N    | Cr   | N    | Percent Cold Reduction | Rockwell C Hardness | Permeability          |         |
|-----------|-----|------|------|------|------|------|------------------------|---------------------|-----------------------|---------|
|           |     |      |      |      |      |      |                        |                     | H = 10                | H = 500 |
| 4321..... | .32 | 13.2 | 0.32 | 0.58 | 8.7  | 0.06 | 10                     | -----               | (strongly) (magnetic) | 1.001   |
| 4322..... | .29 | 13.1 | 0.32 | 0.58 | 8.6  | 0.12 | 0                      | 22                  | 1.014                 | 1.044   |
| 4325..... | .41 | 13.3 | 0.23 | 0.61 | 8.6  | 0.11 | 10                     | 35                  | 1.014                 | 1.314   |
| 4323..... | .27 | 13.5 | 0.32 | 0.62 | 11.9 | 0.17 | 20                     | 41                  | 1.151                 | 1.002   |
| 4326..... | .40 | 13.2 | 0.42 | 0.77 | 12.4 | 0.16 | 0                      | 21                  | 1.121                 | 1.258   |
|           |     |      |      |      |      |      | 10                     | 33                  | 1.018                 | 1.033   |
|           |     |      |      |      |      |      | 20                     | 41                  | 1.121                 | 1.001   |
|           |     |      |      |      |      |      | 0                      | 25                  | 1.001                 | 1.008   |
|           |     |      |      |      |      |      | 10                     | 34                  | 1.001                 | 1.061   |
|           |     |      |      |      |      |      | 20                     | 41                  | 1.035                 | 1.061   |

It is clear from the above that it is necessary to make the 13% manganese steel with carbon over about 0.30%, chromium over about 11%, and nitrogen over about 0.15%, to assure a permeability in the steel less than about 1.2 (for a magnetizing force of H=500 oersteds) after the annealed steel has been cold worked about 20%.

The steel of this invention has satisfactory mechanical properties for general purpose non-magnetic applications as shown in Table II:

TABLE II  
*Mechanical properties of non-magnetic C—Mn—Cr—N steel*

| [Bar 4326 <sup>1</sup> annealed at 1950° F.] |                  |
|----------------------------------------------|------------------|
| 0.2% yield strength                          | 64,000 p. s. i.  |
| Tensile strength                             | 136,000 p. s. i. |
| Elongation                                   | 65%.             |
| Red. of area                                 | 60%.             |
| V-notch Charpy at 80° F.                     | 140 ft. lbs.     |
| V-notch Charpy at minus 40° F.               | 105 ft. lbs.     |
| V-notch Charpy at minus 100° F.              | 75 ft. lbs.      |

<sup>1</sup> Composition given in Table I.

Some applications for such non-magnetic steel are: deck-plates; structural members, such as plates, sheets, I-beams, angles, channels, etc.; or assemblies of such structural members in girders, trusses, engine foundations, fly-wheels, etc. The assemblies can be made either by riveting or welding.

That the composition range above specified for providing the substantially non-magnetic, austenitic steel of the invention is highly critical is evidenced by the following. If the manganese is dropped appreciably below my lower limit of about 11%, while retaining C, Cr and N within my specified limits therefor, the steel nevertheless becomes highly magnetic on quenching. Thus two steels of analysis 0.36C—12Cr—0.17N but containing 7% and 8.6% Mn, respectively, were found to be highly magnetic on aging for 16-32 hours at 1400° F. Other steels containing chromium above my upper limit of 15% were found to be highly magnetic, as solution treated or as solution treated and aged. Thus a steel analyzing about 0.3C—19Cr—12Mn—0.15N was found to be highly magnetic on solution treating at 2100° F. and water quenched. The same was found to be true of other steels analyzing about 0.07/0.3C—23Cr—13Mn—0.6N, and also about 0.25C—29Cr—10Mn—0.25N, the latter being highly magnetic both as solution treated and as subsequently aged at 1400° F. for 2 to 100 hours. This same result was found to be true of steels containing

manganese below and carbon and chromium above my range, such as steels containing about 0.5/0.8C—24Cr—5Mn—0.45N, which were highly magnetic as solution treated at 2100° F. and quenched and thereafter aged 16 hours at 1400° F.

The steel of my invention is not appreciably hardened by an aging heat treatment. Thus a typical steel analyzing about 0.3C—12Cr—11Mn—0.2N had a hardness of 24 Rc (Rockwell "C") as solution treated at 2100° F. and water quenched. On subsequent aging for 8 hours at 1400° F., the hardness had increased only to 28 Rc and to only 31 Rc after 100 hours of aging. This steel was non-magnetic in all conditions of heat treatment.

15 This application is a continuation-in-part of my applications Serial Nos. 349,087, filed April 15, 1953, 414,498, filed March 5, 1954, and 421,997, filed April 9, 1954, all abandoned.

What I claim is:

20 1. An austenitic steel characterized in being substantially non-age hardenable and in having a maximum magnetic permeability of 1.2 with a magnetizing force of about 500 oersteds, both as annealed and after a cold reduction of about 20%, said steel consisting essentially of about: 0.3 to 0.5% carbon, 11 to 15% manganese, 11 to 15% chromium, 0.15 to 0.5% nitrogen, up to 1% each of nickel and silicon, and the balance iron.

25 2. An austenitic steel characterized in being substantially non-age hardenable and in having a maximum magnetic permeability of 1.2 with a magnetizing force of about 500 oersteds, both as annealed and after a cold reduction of about 20%, said steel consisting essentially of about: 0.35 to 0.45% carbon, 13 to 14% manganese, 12 to 13% chromium, 0.15 to 0.25% nitrogen, 0.2 to 0.5% silicon, 0.5 to 1% nickel, and the balance iron.

#### References Cited in the file of this patent

#### UNITED STATES PATENTS

2,696,433 Tanczyn ----- Dec. 7, 1954  
2,698,785 Jennings ----- Jan. 4, 1955

#### FOREIGN PATENTS

152,291 Austria ----- Jan. 5, 1938

#### OTHER REFERENCES

Transaction, American Society for Metals, vol. 41, pages 1306 and 1337. Published in 1949 by the Society.

Making, Shaping and Treating of Steel, sixth edition, pages 12-7-1209. Edited by Camp and Farnsic, published in 1951 by the United States Steel Company, Pittsburgh, Pa.